

March 18, 1941.

L. E. THOMPSON

2,235,051

MANUFACTURE OF SELENIUM AND LIKE RECTIFIERS

Filed Jan. 31, 1940

Fig. 1.



Fig. 2.



Fig. 4.



Fig. 3.



INVENTOR

Leslie Ernest Thompson

BY Kellogg

HIS ATTORNEY.

## UNITED STATES PATENT OFFICE

2,235,051

MANUFACTURE OF SELENIUM AND LIKE  
RECTIFIERS

Leslie Ernest Thompson, King's Cross, London,  
England, assignor, by mesne assignments, to  
The Union Switch and Signal Company, Swiss-  
vale, Pa., a corporation of Pennsylvania

Application January 31, 1940, Serial No. 316,608  
In Great Britain May 26, 1939

## 2 Claims. (Cl. 175—366)

This invention relates to selenium and like rectifiers of the kind comprising a metallic base or support provided with a coating or layer composed of or containing selenium or the like, superposed on which is a counter-electrode or contact layer composed of a suitable metal or alloy, the invention having for its object to provide an improved process of manufacture of rectifiers of this character whereby their production on a relatively large scale may be more conveniently and economically effected than by existing processes.

It has hitherto been customary to manufacture each individual rectifier element separately as regards the preparation of the metallic base and the application thereto of the selenium and contact layers, this process, particularly in the case of small rectifier elements, being relatively slow and expensive.

According to the present invention, however, a base or support of sufficient size to provide a relatively large number of rectifier elements is arranged to be coated as a whole with the required layer of selenium or the like, and subjected to annealing or other treatment, the coated surface of the support being then coated with a contact metal over isolated areas each corresponding to a single rectifier element, the remaining portions of the area of the selenium coating being protected by means of a suitable mask during the application of the metal coating and the coated base thus formed being finally sub-divided by cutting or otherwise at the portions of the selenium coating thus protected.

In order that the nature of the invention may be clearly understood, a preferred process of manufacture embodying the invention will now be briefly described by way of example with reference to the accompanying drawing, Figures 1, 2 and 3, 4 of which are plan views representing various stages in the manufacture of a selenium rectifier in accordance with the invention.

The base or support of which a portion is indicated at 1 in Figures 1 and 3 is constituted by a strip of sheet iron approximately 0.03" thick, the width of the strip corresponding to the width of a single rectifier element, for example 3", the strip being as long as can be conveniently handled, for example, approximately 28".

The upper surface of the metal strip 1 is first roughened by exposing this surface to the action of a sand blast, the strip being preferably arranged to be passed under a sand-blasting nozzle by means of a suitable conveyor.

The metal strips after this treatment may be stored until required, care being taken to keep

their roughened surfaces free from dust, grease and rust.

The next stage in the process of manufacture consists in distributing powdered selenium material evenly over the roughened surface of the metal strip, this material being preferably prepared as described in the specification of my co-pending application for Letters Patent of the United States, Serial No. 316,637, filed on January 31, 1940, for Manufacture of selenium rectifiers. The distribution of the powdered material is preferably effected by a device comprising a hopper containing the material and provided at its lower end with a distributing device comprising a rotating spindle or shaft having suitable slots or grooves in its surface which, during the rotation of the spindle, transfer powdered material from the base of the hopper to an outlet passage containing a gauze diaphragm through which the material falls in a shower or spray on to the surface of the metal strip as the latter passes underneath the outlet. The strip is preferably carried along underneath the distributing device on a suitable conveyor, the driving mechanism of which is geared to the mechanism driving the rotating spindle, arrangements being provided, if desired, for adjusting the relative speed of movement of the conveyor and the spindle so as to regulate the distribution of the powdered material.

The strip with its powdered layer of material then passes into a heated press, preferably hydraulically operated, in which the powdered layer is subjected to a pressure of 750 to 1000 lbs. per sq. inch at a temperature of approximately 120° C. for at least 1 to 1½ minutes.

As a result of this treatment, the powdered material is converted into a relatively hard layer which is firmly adherent to the metal strip, and the latter may be stored, in trays for example, until required for the further stages of the process of manufacture, special care being taken to avoid injury to the coated surface of the strips.

The next stage in the process is the annealing of the rectifier stock formed as above described and for this purpose the coated strips are heated in a suitable annealing furnace to a temperature of approximately 205° C. to 215° C. for a period of from 8 minutes to 40 minutes, the period of maintenance at this temperature being longer the lower the temperature.

The strips are then allowed to cool and the further stages of the process are carried out with as little delay as possible.

The first of these further stages may consist

in immersing the strips in a hot solution of dilute caustic soda, this solution being preferably prepared by dissolving  $\frac{1}{4}$  lb. caustic soda in a gallon of water, the temperatures of the soda bath being from 80° C. to 85° C. After removal from the caustic soda bath, the strips are washed in running water and allowed to drain and to dry. This caustic soda treatment is however, optional and may be omitted if desired.

10 A suitable mask is then applied to the coated surface of each strip, this mask being provided with a number of apertures each corresponding to the effective area of a single rectifier element.

15 The strip attached to or assembled in the mask is then provided with a counter electrode composed of an alloy of tin and cadmium containing approximately from 25% to 60% of cadmium this alloy being applied by a spraying operation preferably effected by means of a suitable metallisation pistol operated at a comparatively low pressure of approximately 30 lbs. per sq. inch.

20 The mask having been removed, the strip which then presents the appearance shown in Figure 1 or 3 in which the metal coating is indicated at 2, is sub-divided into individual rectifier elements by cutting or shearing along the dotted lines indicated at a, b in Figures 1 and 3, these lines being located in the selenium coated portions of the surface of the strip which, having 25 been protected by the mask, are not coated with the metallic alloy. It will be observed that the portions of the strip between the lines, a, b are discarded as waste, the separated rectifier elements being of the larger size shown in Figure 2 30 or of the smaller size shown in Figure 4. Elements of still smaller size may of course be produced in a similar manner by further subdivision of the original strip.

35 When, as is usually the case, the rectifier elements are to be each provided with a central aperture for the purpose of assembly on a rod or bolt, the mask will be of such form as to protect central circular areas 3 for each of the elements eventually formed, and the necessary apertures 4 40 may be punched in these areas at the same time as the strip is sub-divided as above described.

45 The separated rectifier elements may then be subjected to an electrical forming treatment such

for example as that described in the copending application for Letters Patent of the United States, Serial No. 309,040, filed by myself and Alexander Jenkins on December 13, 1939, for Alternating current rectifiers of the selenium type, the rectifier elements being finally tested for current in the forward and reverse directions.

5 It will be understood from the above description that during the earlier stages of the process of manufacture the strip or sheet comprising a large number of rectifier elements is a unit which can be readily handled and treated and it is found that the subsequent sub-division of the strip can be effected without appreciable injury to the selenium coating, while the parts of the surface provided with the superposed metallic layer or coating are unaffected by the cutting or shearing operation, since this is effected at the other portions of the surface.

20 The invention is evidently not limited to the particular process above described by way of example.

Having now particularly described and ascertained the nature of my said invention and in what manner the same is to be performed, I declare that what I claim is:

1. A process for the manufacture of selenium or like rectifiers of the kind described, in which a base or support of sufficient size to provide a relatively large number of rectifier elements is arranged to be coated as a whole with the required layer of selenium or the like, and subjected to annealing or other treatment, the coated surface of the support being then coated with a contact metal or alloy over isolated areas each corresponding to a single rectifier element, the remaining portions of the area of the selenium coating being protected by means of a suitable mask during the application of the metal coating and the coated base thus formed being finally sub-divided by cutting or otherwise at the portions of the selenium coating thus protected, for the purpose specified.

2. A process as claimed in claim 1, in which the final sub-division of the base or support is effected by a double cutting or shearing operation, substantially as described.

LESLIE ERNEST THOMPSON.